

1

2,753,325

## RESINS FROM SELECTED DISTILLATES

Fred W. Banes, Westfield, Joseph F. Nelson, Rahway, and Stanley B. Mirviss, Roselle, N. J., assignors to Esso Research and Engineering Company, a corporation of Delaware

No Drawing. Application December 22, 1952,  
Serial No. 327,438

5 Claims. (Cl. 260—82)

This invention is concerned with the preparation of 15 light-colored, high softening point resins from piperylene containing fractions boiling in the range of 30 to 60° C. which are obtained as selected distillate cuts from steam cracked petroleum streams.

In general, heavier petroleum fractions such as naphtha, gas oil, and the like, are cracked at relatively low pressures and at temperatures of 1000 to 1500° F. in the presence of steam and for relatively short contact times. The gas and liquid streams produced contain large quantities of diolefins and olefins in the C<sub>5</sub> to C<sub>10</sub> range. The naphtha distillate streams obtained by steam cracking operations contain large amounts of diolefins, olefins, aromatics and some paraffins.

In order to obtain the selected polymerization feed streams to be used in this invention, the distillate streams are processed to remove the cyclopentadienes and also the isoprene, if desired.

By using a thermal soaking of the C<sub>5</sub> containing fraction at a temperature of 100 to 250° F. and sufficient heat treating time, the cyclodiienes, mainly the cyclopentadienes, are dimerized and are separated by vacuum- or steam distillation. In this distillation, the hydrocarbons boiling below the dimers are removed as an overhead distillate leaving the dimer-rich residual fraction.

It has now been found that the low-boiling components of this overhead distillate are particularly well suited as feeds for the preparation of light-colored, high softening point resins. The fractions boiling from about 30° C. (the initial boiling point of the fraction) up to 60° are treated with an aluminum halide catalyst at —30° to +70° C. Even higher temperatures may be employed although operating at such temperatures requires pressure equipment. Light yellowish resins can thus be produced in a yield of at least 40% based on the hydrocarbon feed. These resin products have softening points in the range of 75° to 100° C. The volatile, unpolymerized components recovered from the polymerization step can be used as feed stock for oxonation reactions, if desired, to produce valuable aldehydes and alcohols; for hydration to alcohols and for alkylating aromatics.

The preferred feed stocks are fractions boiling from 30° to 60° C., and are relatively free of cyclopentadienes. It is particularly desirable that at least 40% of the polymerization feed comprises components boiling in the range of 38° to 46° C. Various cuts within 30° to 60° range can be used as long as the piperylene concentration of the cut is within a certain specified range, particularly about 15 to not more than about 60 volume per cent. The following table shows characteristic compositions of these distillate streams:

| Component:                                | Vol. per cent |
|-------------------------------------------|---------------|
| Isoprene                                  | 15-0          |
| Piperylenes                               | 15-60         |
| C <sub>5</sub> acyclic and cyclic olefins | 70-35         |
| Paraffins and naphthenes                  | 0-3           |
| C <sub>6</sub> +                          | 0-2           |

2

Specific examples of cuts which are satisfactory are shown below. One cut shown which contains 73% piperylene is unsatisfactory as resin feed.

| 5 Feed No.                       | 1     | 2     | 3     | 4     | 5     |
|----------------------------------|-------|-------|-------|-------|-------|
| Distillation Range, ° C.         | 30-60 | 30-48 | 35-48 | 38-46 | 38-46 |
| Vol. Percent in 38°-46° C. Range | 50    | 60    | 75    | 96    | 92    |
| Feed                             | (3)   | (3)   | (3)   | (3)   | (4)   |
| Vol. Percent Piperylene          | 15    | 20    | 38    | 54    | 73    |
| Vol. Percent Isoprene            | 14    | 15    | 14    | 1     | 3.5   |

<sup>3</sup> Satisfactory.

<sup>4</sup> Unsatisfactory.

|                          | Volume Percent |     |
|--------------------------|----------------|-----|
| Isoprene                 | (1)            | (2) |
| t-Piperylene             | 1              | 3.5 |
| cis-Piperylene           | 39             | 63  |
| Cyclopentene             | 15             | 10  |
| C <sub>5</sub> Olefins   | 15             | 9   |
| C <sub>6</sub> Saturates | 27             | 13  |
| C <sub>6</sub> +         | 2              | <1  |
|                          | 1              | 1.5 |

25 The reactive components in the stream are polymerized in the presence of an aluminum halide catalyst. Aluminum chloride and aluminum bromide can be used either in the solid or powdered form or as slurries in inert diluents. Solubilized aluminum halide catalysts are also 30 quite satisfactory and are preferred for giving the best C<sub>6</sub>-free products. Also, the aluminum halide may be added in the form of a complex. If desired, the complex 35 may be formed by interaction of AlCl<sub>3</sub> with the unreacted hydrocarbons stripped from resin product or from naphthas containing olefins and aromatics. As one 40 illustration a naphtha containing about 60% olefins and 40% aromatics is satisfactory. Preferred catalyst concentrations are in the range of 0.25 to 2.5% based on the hydrocarbon feed. The reaction is carried out at temperatures in the range of —30 to +70° C., preferably 45 —10 to +55° C. A diluent may be used if desired.

The polymerization reaction is carried out as a liquid 50 phase operation. The catalyst may be added continually or batchwise. Any practical and effective methods for adding catalyst and reagents can be utilized. The time required to carry out the reaction depends primarily on the rate that the catalyst can be added that will allow adequate control of the reaction temperature. The reaction products are worked up by water or caustic washing or by washing with dilute H<sub>2</sub>SO<sub>4</sub> (5%) followed by 55 water washing. The catalyst residues can also be removed by precipitation as a methanol catalyst complex followed by subsequent filtration. The latter process provides for removal of any insoluble polymer formed during the course of the polymerization. The polymerized reaction product is then stripped free of unreacted components of the feed and low molecular weight polymerization products to give the final resin.

The yield and softening point of the final resin will 60 depend on the degree of stripping. Stripping to a pot temperature of 200-300° C. at 1-50 mm. Hg, preferably 240-270° C. at 1 to 5 mm. Hg has given acceptable resin products. Steam stripping at temperatures of 250-270° C. can also be employed to produce high softening point resins.

65 The resins are compatible with and can be readily co-bodied with non-conjugated drying oils at linseed, soya and the like. Although the bodying rate with highly conjugated oils as tung or oiticica is very rapid, the resins can be used satisfactorily with linseed-tung oil blends or soya-oiticica, etc. to give excellent varnishes. These varnishes can be prepared by cooking at temperatures as

high as 550° F. without encountering insolubilization. Cooking losses are low, e. g. 6% or less. The varnishes are especially useful for can coating applications because of their excellent flexibility and chemical resistance characteristics. Baked films prepared from cobodied solid resins and a 50/50 linseed/tung mixture (20 lbs. resin/100 gallons of oil) show no failures upon bending (as in can forming operations). The resins are also suitable for use in printing ink formulations.

feeds having up to about 55-60% of piperylene (the remainder of the feed being largely olefinic) are satisfactory as resin feed streams, giving good yields of resins of high softening point, light color, and low iodine number with relatively small amounts of insoluble polymer. The olefinic feed having more than about 60% of piperylene gave a greatly decreased yield of soluble resin having a low softening point and large amounts of insoluble polymer. Details are shown in Table II below.

Table II

| Feed Boiling Range, ° C. | Vol. percent 1,3-Penta-diene (piperylene) in Feed | Percent Catalyst       | Wt. percent |                | Resin Properties |       |               |
|--------------------------|---------------------------------------------------|------------------------|-------------|----------------|------------------|-------|---------------|
|                          |                                                   |                        | Sol. Resin  | Insol. Polymer | Soft. Pt., ° C.  | Color | Iodine Number |
| 30-48                    | 20                                                | 1% AlCl <sub>3</sub>   | 49.2        | 9.8            | 77               | 0     | 235           |
| 30-48                    | 20                                                | 1% AlCl <sub>3</sub> * | 57.2        | None           | 78               | 1     | 209           |
| 35-46                    | 54                                                | 1% AlCl <sub>3</sub>   | 68.3        | 2.3            | 84               | 0     | 209           |
| 38-46                    | 54                                                | 1% AlCl <sub>3</sub> * | 65.5        | None           | 78               | 1     | 215           |
| 38-46                    | 54                                                | 1% AlBr <sub>3</sub>   | 65.0        | 2.0            | 84               | 0     | 215           |
| 38-46                    | 73                                                | 0.7% AlCl <sub>3</sub> | 35.8        | 22             | <25              | 1     | 255           |

\*Added as a soluble liquid hydrocarbon complex. Complex prepared by adding solid AlCl<sub>3</sub> to a mixture of C<sub>5</sub>-C<sub>8</sub> olefins (60%), benzene (30%) and toluene (10%).

The invention will be described in greater detail by the following examples:

## EXAMPLE 1

A steam cracked distillate stream was subjected to a thermal treatment to dimerize the cyclodienes. These cyclodiene dimers were then removed by careful fractionation as a bottoms stream. The lighter portions were obtained as an overhead stream.

The overhead from the cyclopentadiene recovery operation was fractionated to obtain a cut boiling in the range of about 30 to 60° C. This cut contained about 15% 1,3-pentadiene (piperylene). Samples of this distillate fraction were then treated with AlCl<sub>3</sub> or with BF<sub>3</sub> at reaction temperatures in the range of 0° up to about 25° C. The reaction products were then water washed or treated with CH<sub>3</sub>OH to remove residual catalyst, filtered and then stripped to a bottoms (resin) temperature of 270° C. at 3-4 mm. Hg. Specific data are shown in Table I below:

Table I

| Catalyst          |                 | Reaction Temp., ° C. | Yield, Wt. Percent |                   | Resin Properties             |                    |                         |            |
|-------------------|-----------------|----------------------|--------------------|-------------------|------------------------------|--------------------|-------------------------|------------|
| Type              | Amount, Percent |                      | Soluble Resin      | Insoluble Product | Soft. Pt., ° C. <sup>1</sup> | Color <sup>2</sup> | Iodine No. <sup>3</sup> | Int. Visc. |
| AlCl <sub>3</sub> | 0.67            | 8-10                 | 61.2               | 4.8               | 76                           | 0                  | 238                     | .058       |
| AlCl <sub>3</sub> | 0.66            | 10-15                | 56.3               | 6.2               | 79                           | 1                  | 192                     | —          |
| AlCl <sub>3</sub> | 1.0             | 10-15                | 49.2               | 6.8               | 88                           | 0                  | 235                     | .066       |
| AlCl <sub>3</sub> | 0.61            | 15-20                | 43.3               | 3.2               | 82                           | 1                  | 184                     | —          |
| AlCl <sub>3</sub> | 1.0             | 15-20                | 48.4               | 5.5               | 79                           | 0                  | 225                     | .058       |
| BF <sub>3</sub>   | 0.3             | 0                    | 41.5               | —                 | <25                          | 1                  | —                       | —          |
| BF <sub>3</sub>   | 0.67            | 15-20                | 48.5               | —                 | <25                          | 0                  | 250                     | .029       |

<sup>1</sup> Ring and ball method (ASTM E-28-51-T).

<sup>2</sup> Color of solution of 1 g. resin in 67 ml. xylenes compared to Gardner color index.

<sup>3</sup> ASTM (D-555-47).

The comparative data shown above indicate the great advantages obtained in preparing resins by this invention. The soluble resin is produced in good yield with relatively small amounts of insoluble gelled product. The AlCl<sub>3</sub> catalyst produced a resin having a softening point well above 75° C., and a very light color. The BF<sub>3</sub> resin, however, has a softening point of less than 25° C. and a somewhat higher unsaturation (as indicated by the iodine number).

## EXAMPLE 2

A series of experiments similar to that described in Example 1 was carried out. The distillate feed stream was varied somewhat, the percentage of piperylene varying from 20 to 73%. These comparative experiments show

## EXAMPLE 3

A steam cracked distillate stream boiling from 38-46° C. and containing 54% piperylene and about 42% C<sub>5</sub> olefins was polymerized with AlCl<sub>3</sub> at temperatures varying from -10° to +35° C. The resin products were of uniformly good quality. The data of the experiments are shown in Table III.

Table III

| Wt. Percent Catalyst | Reaction Temp., ° C. | Yield, Wt. Percent |                | Resin Properties |       |               |  |
|----------------------|----------------------|--------------------|----------------|------------------|-------|---------------|--|
|                      |                      | Sol. Resin         | Insol. Polymer | Soft. Pt., ° C.  | Color | Iodine Number |  |
| 0.5                  | 20                   | 62.7               | 2.5            | 77               | 0     | 220           |  |
| 2.0                  | 20                   | 69.5               | 2.5            | 84               | 0     | 200           |  |
| 1.0                  | -10                  | 62.3               | 2.2            | 78               | 0     | 207           |  |
| 1.0                  | 20                   | 68.3               | 2.3            | 84               | 0     | 209           |  |
| 1.0                  | 35                   | 65.0               | 2.2            | 84               | 0     | 221           |  |

## EXAMPLE 4

In another series of polymerizations, a fraction of steam cracked distillate boiling in the range of about 36 to 48° C. and containing approximately 38 volume percent piperylene and 14 volume percent isoprene was used as the feed. Various catalysts or catalyst mixtures were added to samples of the feed, in each case using 1% catalyst at a reaction temperature of 15-20° C. The reaction products were quenched with a 5% H<sub>2</sub>SO<sub>4</sub> solution, water washed thoroughly and then stripped to a bottoms temperature of 270° C. at 5 mm. Hg to recover light colored solid resins. The detailed data are shown in Table IV.

**5**  
*Table IV*

| Catalyst                | Method of Add'n                             | Yield, Wt. Percent |                | Soluble Resin Properties |       |
|-------------------------|---------------------------------------------|--------------------|----------------|--------------------------|-------|
|                         |                                             | Sol. Resin         | Insol. Polymer | Soft. Pt., °C.           | Color |
| AlCl <sub>3</sub> ..... | 5.8 wt. Percent Solution in Ethyl Chloride. | 72.2               | None           | 88                       | 0     |
| AlBr <sub>3</sub> ..... | 6.3 wt. percent Solution in n-hexane.       | 70.6               | None           | 88                       | ½     |
| AlCl <sub>3</sub> ..... | Solid 30 Mesh.....                          | 68.3               | 2.4            | 84                       | 0     |

These data show that solution of aluminum catalysts can be used to give high yields of excellent quality and completely soluble resins.

#### EXAMPLE 5

The steam cracked distillate fraction described in Example 4 above was diluted with n-heptane to give a solution containing 62.5% of the unsaturated fraction. This solution was polymerized at 55° C. using 1% AlBr<sub>3</sub>. The catalyst was added as a 6% solution in n-heptane over a period of ½ hour and the reaction mixture was held at 55° C. for an additional ½ hour with agitation. The reaction mixture was then quenched by the addition of 75 ml. of 5% H<sub>2</sub>SO<sub>4</sub>, water washed and then stripped to a bottoms (resin) temperature of 280° C. at 5 mm. Hg. The completely soluble resin product had a Gardner color of ½, a softening point of 98° C., and represented a yield of 69.2 wt. percent on the distillate portion of the polymerization feed.

What is claimed is:

1. A process for the preparation of soluble hydrocarbon resins having Gardner colors of about 0-1 which comprises subjecting a C<sub>5</sub> fraction from a steam cracked petroleum stream containing about 15-60 volume percent piperylene and about 35-70 volume percent olefins

to thermal soaking at a temperature of about 37° to 122° C. for a sufficient time to dimerize the cyclodienes, separating the fraction boiling between about 30 and 60° C. from the dimers, subjecting the undimerized portion to polymerization in the presence of aluminum halide catalyst until a yield of at least about 43 wt. percent soluble resins are obtained, and recovering the resins formed in the absence of alkalies.

2. A process according to claim 1 in which the undimerized portion is fractionated into a fraction boiling between 38 and 46° C. and is subjected to polymerization with aluminum chloride at a temperature between -10 and +55° C.

3. A process according to claim 2 in which the fraction boiling between 30 and 60° C. is subjected to polymerization in the presence of 0.25 and 2.5% of aluminum chloride the polymerization being continued until a yield of above about 60 wt. percent soluble resin having a Gardner color of about 0-1 is obtained.

4. A process according to claim 1 in which at least 40 per cent of the 30 to 60° C. fraction boils in the range of 38 to 46° C., which 40 per cent contains from 15 to 55 volume per cent of piperylene.

5. A process according to claim 1 in which the undimerized portion is separated into a fraction boiling from 48 to 36° C. having from 48 to 54 volume per cent of piperylene and is subjected to polymerization in the presence of a solubilized aluminum halide catalyst at a temperature between -10 and +55° C. until a yield of at least about 70 wt. percent soluble resin is obtained.

#### References Cited in the file of this patent

##### UNITED STATES PATENTS

- |    |           |                     |               |
|----|-----------|---------------------|---------------|
| 35 | 1,982,708 | Thomas et al. ----- | Dec. 4, 1934  |
|    | 2,062,845 | Thomas et al. ----- | Dec. 1, 1936  |
|    | 2,271,636 | Frolich -----       | Feb. 3, 1942  |
|    | 2,521,022 | Rowland -----       | Sept. 5, 1950 |